



particles are composed of either one or both of metallic titanium powder particles and hydrogenated titanium powder particles.

(56)

**References Cited**

## U.S. PATENT DOCUMENTS

2012/0094142 A1 4/2012 Hoshino et al.  
2012/0135142 A1 5/2012 Yang et al.

**8 Claims, 8 Drawing Sheets****(51) Int. Cl.**

**B22F 3/10** (2006.01)  
**B22F 3/11** (2006.01)  
**C22C 1/08** (2006.01)  
**C22C 21/00** (2006.01)  
**C22C 1/04** (2006.01)  
**C22C 47/14** (2006.01)  
**B22F 7/00** (2006.01)  
**C22C 49/14** (2006.01)

**(52) U.S. Cl.**

CPC ..... **B22F 1/025** (2013.01); **B22F 3/11** (2013.01); **B22F 7/002** (2013.01); **C22C 1/0416** (2013.01); **C22C 1/08** (2013.01); **C22C 21/00** (2013.01); **C22C 21/003** (2013.01); **C22C 47/14** (2013.01); **C22C 49/14** (2013.01)

**(58) Field of Classification Search**

CPC ..... B22F 3/1003; B22F 3/11; B22F 7/002; C22C 1/0416; C22C 1/08; C22C 21/00; C22C 21/003; C22C 47/14; C22C 49/14

See application file for complete search history.

(56)

## FOREIGN PATENT DOCUMENTS

|    |                  |                           |
|----|------------------|---------------------------|
| CN | 102305564 A      | 1/2012                    |
| EP | 2939762 A        | 11/2015                   |
| EP | 2962791 A        | 1/2016                    |
| JP | 61084351 A       | * 4/1986 ..... C22C 32/00 |
| JP | 08-325661 A      | 12/1996                   |
| JP | 2009-256788 A    | 11/2009                   |
| JP | 2010-280951 A    | 12/2010                   |
| JP | 2011-023430 A    | 2/2011                    |
| JP | 2011-077269 A    | 4/2011                    |
| JP | 2011-175934 A    | 9/2011                    |
| JP | 2011-214049 A    | 10/2011                   |
| JP | 2012-507464 A    | 3/2012                    |
| JP | 2012-195182 A    | 10/2012                   |
| WO | WO-2010/051292 A | 5/2010                    |
| WO | WO-2010/116679 A | 10/2010                   |

## OTHER PUBLICATIONS

Office Action dated May 3, 2016 for the corresponding Chinese Patent Application No. 201480004359.4.

Office Action dated Dec. 30, 2016 for the corresponding Chinese Patent Application No. 201480004359.4.

Extended European Search Report dated Jul. 19, 2016 for the corresponding European Patent Application No. 14756420.7.

\* cited by examiner

FIG. 1



FIG. 2



FIG. 3



FIG. 4



FIG. 5



FIG. 6



FIG. 7





FIG. 8

**ALUMINUM MATERIAL FOR SINTERING,  
METHOD FOR PRODUCING ALUMINUM  
MATERIAL FOR SINTERING, AND  
METHOD FOR PRODUCING POROUS  
ALUMINUM SINTERED COMPACT**

**CROSS-REFERENCE TO RELATED PATENT  
APPLICATIONS**

This application is a U.S. National Phase Application under 35 U.S.C. § 371 of International Patent Application No. PCT/JP2014/054876, filed Feb. 27, 2014, and claims the benefit of Japanese Patent Applications No. 2013-040877, filed Mar. 1, 2013 and No. 2014-028874, filed Feb. 18, 2014, all of which are incorporated by reference in their entirety herein. The International Application was published in Japanese on Sep. 4, 2014 as International Publication No. WO/2014/133079 under PCT Article 21(2).

**FIELD OF THE INVENTION**

The present invention relates to an aluminum material for sintering (aluminum sintering material, aluminum material to be sintered, aluminum raw sintering material) that is used for producing a porous aluminum sintered compact in which a plurality of aluminum base materials are sintered together, a method for producing the aluminum sintering material, and a method for producing a porous aluminum sintered compact in which the aluminum sintering material is used.

**BACKGROUND OF THE INVENTION**

The above-described porous aluminum sintered compact is used for, for example, electrodes and current collectors in a variety of batteries, heat exchanger components, silencing components, filters, impact-absorbing components, and the like.

In the related art, the above-described porous aluminum sintered compact is produced using, for example, the methods disclosed by Patent Documents 1 to 5.

In Patent Document 1, a mixture is formed by mixing aluminum powder, paraffin wax particles, and a binder, and the mixture is shaped into a sheet shape. This mixture is naturally dried. Next, the mixture is immersed in an organic solvent so as to remove the wax particles, subsequently, drying, defatting, and sintering are carried out; and thereby, a porous aluminum sintered compact is produced.

In addition, in Patent Documents 2 to 4, aluminum powder, sintering aid powder containing titanium, a binder, a plasticizer, and an organic solvent are mixed together so as to form a viscous composition, and the viscous composition is shaped and foamed. Then, the viscous composition is heated and sintered in a non-oxidizing atmosphere; and thereby, a porous aluminum sintered compact is produced.

Furthermore, in Patent Document 5, base powder consisting of aluminum, Al alloy powder used to form bridging portions which contains a eutectic element, and the like are mixed together and the mixture is heated and sintered in a hydrogen atmosphere or a mixed atmosphere of hydrogen and nitrogen; and thereby, a porous aluminum sintered compact is produced. Meanwhile, this porous aluminum sintered compact has a structure in which the particles of the base powder consisting of aluminum are connected together through bridging portions having a hypereutectic structure.

Meanwhile, in the porous aluminum sintered compact and the method for producing the porous aluminum sintered compact described in Patent Document 1, there has been a

problem in that it is difficult to obtain a porous aluminum sintered compact having high porosity. Furthermore, in the case in which the aluminum base materials are sintered together, the bonding between the aluminum base materials is hindered by oxide films formed on the surfaces of the aluminum base materials and there has been a problem in that it is not possible to obtain a porous aluminum sintered compact having sufficient strength.

In addition, in the porous aluminum sintered compact and the method for producing the porous aluminum sintered compact described in Patent Documents 2 to 4, there has been a problem in that, since the viscous composition is shaped and foamed, it is not possible to efficiently produce a porous aluminum sintered compact. Furthermore, there has been another problem in that, since the viscous composition contains a large amount of a binder, a long period of time is required for a binder removal treatment, the shrinkage ratio of the compact becomes large during sintering, and it is not possible to produce a porous aluminum sintered compact with excellent dimensional accuracy.

Furthermore, in the porous aluminum sintered compact and the method for producing the porous aluminum sintered compact described in Patent Document 5, there is provided a structure in which the particles of the base powder consisting of aluminum are bonded together through the bridging portions having a hypereutectic structure. In this structure, Al alloy powder having a eutectic composition and a low melting point is melted so as to generate a liquid phase and the liquid phase is solidified among the base powder particles; and thereby, the bridging portions are formed. Therefore, it has been difficult to obtain a porous aluminum sintered compact having high porosity.

**PRIOR ART DOCUMENTS**

Patent Documents

Patent Document 1: Japanese Unexamined Patent Application, First Publication No. 2009-256788

Patent Document 2: Japanese Unexamined Patent Application, First Publication No. 2010-280951

Patent Document 3: Japanese Unexamined Patent Application, First Publication No. 2011-023430

Patent Document 4: Japanese Unexamined Patent Application, First Publication No. 2011-077269

Patent Document 5: Japanese Unexamined Patent Application, First Publication No. H08-325661

**SUMMARY OF THE INVENTION**

Problems to be Solved by the Invention

The present invention has been made in consideration of the above-described circumstances and the present invention aims to provide an aluminum sintering material that makes it possible to efficiently produce, at low cost, a high-quality porous aluminum sintered compact having a small shrinkage ratio during sintering, excellent dimensional accuracy, and sufficient strength, a method for producing the aluminum sintering material, and a method for producing a porous aluminum sintered compact in which the aluminum sintering material is used.

**Means for Solving the Problem**

In order to solve the above-described problems and achieve the above-described object, the aluminum sintering

material of the present invention is an aluminum sintering material that is used for producing a porous aluminum sintered compact in which a plurality of aluminum base materials are sintered together, the aluminum sintering material includes: the aluminum base materials; and a plurality of titanium powder particles fixed to outer surfaces of the aluminum base materials, wherein the titanium powder particles are composed of either one or both of metallic titanium powder particles and hydrogenated titanium powder particles.

In the case in which the aluminum sintering material of the present invention provided with the above-described features is heated at a temperature near the melting point of aluminum during sintering, the aluminum base materials are melted. However, since oxide films are formed on the surfaces of the aluminum base materials, the molten aluminum is held by the oxide films and the shapes of the aluminum base materials are maintained. The oxide films are broken by the reaction with titanium powder particles which are fixed to the surfaces of the aluminum base materials, the molten aluminum inside the aluminum sintering material is ejected outwards, and the ejected molten aluminum reacts with titanium and thus a compound having a higher melting point is generated and solidified. Thereby, a plurality of columnar protrusions protruding outwards are formed on the outer surfaces of the aluminum base materials.

In addition, since the aluminum base materials are bonded together through the columnar protrusions formed on the outer surfaces of the aluminum base materials, it is possible to obtain a porous aluminum sintered compact having high porosity without separately carrying out a foaming step and the like. Therefore, it becomes possible to efficiently produce a porous aluminum sintered compact at low cost.

Furthermore, unlike when a viscous composition is used, a large amount of a binder is not present between the aluminum base materials; and therefore, the shrinkage ratio during sintering is small and it becomes possible to obtain a porous aluminum sintered compact having excellent dimensional accuracy.

In addition, since the oxide films are broken by titanium, the aluminum base materials can be reliably bonded together and it is possible to obtain a porous aluminum sintered compact having sufficient strength.

Furthermore, since the molten aluminum is solidified by titanium, it is possible to prevent the gaps between the aluminum base materials from being filled with the molten aluminum and it is possible to obtain a porous aluminum sintered compact having high porosity.

Here, the amount of the titanium powder particles is preferably set to be in a range of 0.5 mass % to 20 mass %.

In this case, since the amount of the titanium powder particles is set to be in a range of 0.5 mass % or more, the columnar protrusions are sufficiently formed on the outer surfaces of the aluminum base materials, the aluminum base materials can be reliably bonded together, and it is possible to obtain a porous aluminum sintered compact having sufficient strength. In addition, since the amount of the titanium powder particles is set to be in a range of 20 mass % or less, the columnar protrusions are not formed on the outer surfaces of the aluminum base materials more than necessary (a minimal amount of columnar protrusions are formed on the outer surfaces of the aluminum base materials) and it is possible to ensure high porosity.

Furthermore, the aluminum base materials are preferably composed of either one or both of aluminum fibers and aluminum powder.

In the case in which aluminum fibers are used as the aluminum base materials, it is easy to maintain gaps when the aluminum fibers are bonded together through the columnar protrusions, and there is a tendency for the porosity to increase. Therefore, when aluminum fibers and aluminum powder are used as the aluminum base materials and the mixing ratio thereof is adjusted, it becomes possible to control the porosity of the porous aluminum sintered compact.

10 The method for producing an aluminum sintering material of the present invention is a method for producing the above-described aluminum sintering material, the method includes: a mixing step of mixing the aluminum base materials and the titanium powder with a binder; and a 15 drying step of drying a mixture obtained in the mixing step.

According to the method for producing an aluminum sintering material having the above-described features, since the mixing step of mixing the aluminum base materials and the titanium powder with a binder and the drying step of 20 drying a mixture obtained in the mixing step are included, the titanium powder particles are dispersed and fixed to the outer surfaces of the aluminum base materials and the above-described aluminum sintering material is produced.

Here, the drying step is preferably either one of low- 25 temperature drying conducted at a temperature of 40°C. or lower or reduced-pressure drying conducted at a pressure of 1.33 Pa or less.

30 In this case, in the drying step, it is possible to suppress (limit) the forming of thick oxide films on the surfaces of the aluminum base materials, and the sinterability of the aluminum sintering material can be improved.

In addition, the method for producing a porous aluminum sintered compact of the present invention is a method for producing a porous aluminum sintered compact in which the 35 above-described aluminum sintering material is used, the method includes: a material distributing step of distributing the aluminum sintering material to a holding body; and a sintering step of heating and sintering the aluminum sintering material held by the holding body.

40 According to the method for producing a porous aluminum sintered compact having the above-described features, since the above-described aluminum sintering material is used, the oxide films on the aluminum base materials are broken by the titanium powder particles fixed to the outer 45 surfaces of the aluminum base materials during sintering and the molten aluminum inside the aluminum base materials is ejected outwards. The molten aluminum reacts with titanium and thus a compound having a higher melting point is generated and solidified. Thereby, a plurality of columnar protrusions protruding outwards are formed on the outer surfaces of the aluminum base materials.

In addition, a plurality of the aluminum base materials are bonded together through the columnar protrusions and it is possible to produce a porous aluminum sintered compact 55 having high porosity and sufficient strength.

#### Effects of the Invention

According to the present invention, it is possible to 60 provide an aluminum sintering material that makes it possible to obtain a high-quality porous aluminum sintered compact, a method for producing the aluminum sintering material, and a method for producing a porous aluminum sintered compact in which the aluminum sintering material is used. By using the aluminum sintering material of the present invention, it is possible to efficiently produce a 65 porous aluminum sintered compact at low cost, and the

produced porous aluminum sintered compact has a small shrinkage ratio during sintering, excellent dimensional accuracy, and sufficient strength.

#### BRIEF DESCRIPTION OF THE DRAWINGS

FIG. 1 shows a porous aluminum sintered compact produced using an aluminum sintering material which is an embodiment of the present invention. FIG. 1(a) is an observation photograph of the porous aluminum sintered compact and FIG. 1(b) is a schematic enlarged view of the porous aluminum sintered compact.

FIG. 2 shows a joining portion between aluminum base materials in the porous aluminum sintered compact shown in FIG. 1. FIGS. 2(a) and 2(b) are SEM observation photographs of the joining portion, FIG. 2(c) is a composition analysis result showing an Al distribution in the joining portion, and FIG. 2(d) is a composition analysis result showing a Ti distribution in the joining portion.

FIG. 3 shows an aluminum sintering material which is the embodiment of the present invention. FIGS. 3(a) and 3(b) are SEM observation photographs of the aluminum sintering material, FIG. 3(c) is a composition analysis result showing an Al distribution in the aluminum sintering material, and FIG. 3(d) is a composition analysis result showing a Ti distribution in the aluminum sintering material.

FIG. 4 is a flowchart showing an example of a method for producing the aluminum sintering material which is an embodiment of the present invention and a method for producing the porous aluminum sintered compact shown in FIG. 1.

FIG. 5 shows the aluminum materials for sintering according to the present embodiment in which titanium powder particles are fixed to outer surfaces of aluminum base materials. FIG. 5(a) shows the aluminum sintering material in which the aluminum base material is an aluminum fiber and FIG. 5(b) shows the aluminum sintering material in which the aluminum base material is aluminum powder.

FIG. 6 is a schematic explanatory view of a continuous sintering device used to produce a sheet-shaped porous aluminum sintered compact.

FIG. 7 shows a state in which columnar protrusions are formed on the outer surfaces of the aluminum base material in a sintering step. FIG. 7(a) shows the case in which the aluminum base material is an aluminum fiber and FIG. 7(b) shows the case in which the aluminum base material is aluminum powder.

FIG. 8 is an explanatory view showing a production step of producing a bulk-shaped porous aluminum sintered compact.

#### DETAILED DESCRIPTION OF THE INVENTION

Hereinafter, an aluminum sintering material, a method for producing the aluminum sintering material, and a method for producing a porous aluminum sintered compact in which the aluminum sintering material is used, which are embodiments of the present invention, will be described.

First, a porous aluminum sintered compact 10 produced using the aluminum sintering material according to the present embodiment will be described.

FIG. 1 shows a porous aluminum sintered compact 10 produced using an aluminum sintering material according to the present embodiment. FIG. 1(a) is an observation photograph of the porous aluminum sintered compact according

to the present embodiment, and FIG. 1(b) is a schematic view of the porous aluminum sintered compact according to the present embodiment.

As shown in FIG. 1, the porous aluminum sintered compact 10 is obtained by integrating a plurality of aluminum base materials 11 through sintering and the porosity is set to be in a range of 30% to 90%.

In the present embodiment, as shown in FIG. 1, aluminum fibers 11a and aluminum powder (aluminum powder particles) 11b are used as the aluminum base materials 11.

In addition, a plurality of columnar protrusions 12 protruding outwards are formed on the outer surfaces of the aluminum base materials 11 (the aluminum fibers 11a and the aluminum powder 11b), and a structure is provided in which a plurality of the aluminum base materials 11 and 11 (the aluminum fibers 11a and the aluminum powder 11b) are bonded together through the columnar protrusions 12. As shown in FIG. 1, bonding portions 15 between the aluminum base materials 11 and 11 include portions at which the columnar protrusions 12 and 12 are bonded together, portions at which the columnar protrusion 12 and the side surface of the aluminum base material 11 are joined together, and portions at which the side surfaces of the aluminum base materials 11 and 11 are joined together.

As shown in FIG. 2, a Ti—Al-based compound 16 is present in the bonding portion 15 between the aluminum base materials 11 and 11 that are bonded together through the columnar protrusion 12. In the present embodiment, as shown in the analysis result of FIG. 2, the Ti—Al-based compound 16 is a compound of Ti and Al and, more specifically, the Ti—Al-based compound 16 is an  $Al_3Ti$  intermetallic compound. That is, in the present embodiment, the aluminum base materials 11 and 11 are bonded together at portions in which the Ti—Al-based compound 16 is present.

Next, an aluminum sintering material 20 according to the present embodiment will be described.

As shown in FIG. 3, the aluminum sintering material 20 includes the aluminum base materials 11 and a plurality of titanium powder particles 22 fixed to the outer surface of the aluminum base material 11. Meanwhile, as the titanium powder particles 22, either one or both of metallic titanium powder particles and hydrogenated titanium powder particles can be used.

In the aluminum sintering material 20, the amount of the titanium powder particles 22 is set to be in a range of 0.5 mass % to 20 mass %, preferably in a range of 0.5 mass % to 15 mass %, and still more preferably in a range of 1.0 mass % to 10 mass %. In the present embodiment, the amount thereof is set to 5 mass %.

In addition, the particle diameters of the titanium powder particles 22 are set to be in a range of 1  $\mu m$  to 50  $\mu m$  and 55 preferably set to be in a range of 5  $\mu m$  to 30  $\mu m$ . In addition, since it is possible to make the particle diameters of the hydrogenated titanium powder particles smaller than those of the metallic titanium powder particles, the hydrogenated titanium powder particles are preferably used in the case in which it is necessary to decrease the particle diameters of the titanium powder particles 22 that are fixed to the outer surfaces of the aluminum base materials 11.

Furthermore, the intervals between the titanium powder particles 22 and 22 fixed to the outer surface of the aluminum base material 11 are preferably set to be in a range of 5  $\mu m$  to 100  $\mu m$  and more preferably set to be in a range of 5.0  $\mu m$  to 70  $\mu m$ .

As the aluminum base materials **11**, as described above, the aluminum fibers **11a** and the aluminum powder **11b** are used. As the aluminum powder **11b**, atomized powder can be used.

The fiber diameters of the aluminum fibers **11a** are set to be in a range of 40  $\mu\text{m}$  to 300  $\mu\text{m}$  and preferably set to be in a range of 50  $\mu\text{m}$  to 200  $\mu\text{m}$ . In addition, the fiber lengths of the aluminum fibers **11a** are set to be in a range of 0.2 mm to 20 mm and preferably set to be in a range of 1 mm to 10 mm.

In addition, the particle diameters of the aluminum powder **11b** are set to be in a range of 20  $\mu\text{m}$  to 300  $\mu\text{m}$  and preferably set to be in a range of 20  $\mu\text{m}$  to 100  $\mu\text{m}$ .

Furthermore, the aluminum base materials **11** are preferably made of pure aluminum having a purity of 99.5 mass % or more and, furthermore, the aluminum base materials **11** are preferably made of 4N aluminum having a purity of 99.99 mass % or more.

In addition, it becomes possible to adjust the porosity by adjusting the mixing ratio between the aluminum fibers **11a** and the aluminum powder **11b**. That is, when the ratio of the aluminum fibers **11a** is increased, it becomes possible to increase the porosity of the porous aluminum sintered compact **10**. Therefore, as the aluminum base materials **11**, the aluminum fibers **11a** are preferably used and, in the case in which the aluminum powder **11b** is mixed, the ratio of the aluminum powder **11b** is preferably set to be in a range of 10 mass % or less and more preferably set to be in a range of 1.0 mass % to 5.0 mass %.

Next, a method for producing an aluminum sintering material and a method for producing a porous aluminum sintered compact, which are the present embodiments, will be described with reference to the flowchart of FIG. 4.

First, as shown in FIG. 4, the aluminum sintering material **20** according to the present embodiment is produced.

The aluminum base materials **11** and titanium powder are mixed together at normal temperature (Mixing Step **S01**). At this time, a binder solution is sprayed. As the binder, a binder that is combusted and decomposed when heated at 500°C. in air atmosphere is preferable and, specifically, an acryl-based resin or a cellulose-based macromolecular body is preferably used. In addition, as a solvent for the binder, a variety of solvents such as water-based solvents, alcohol-based solvents, and organic solvents can be used.

In the Mixing Step **S01**, the aluminum base materials **11** and the titanium powder are mixed while being made to flow using a variety of mixers such as an automatic mortar, a pan-type tumbling granulator, a shaker mixer, a pot mill, a high-speed mixer, and a V-type mixer.

Next, a mixture obtained in the Mixing Step **S01** is dried (Drying Step **S02**). In the Drying Step **S02**, the mixture is subjected to drying at a low temperature of 40°C. or lower or drying at a reduced pressure of 1.33 Pa or less (10<sup>-2</sup> Torr or less) so as to prevent thick oxide films from being formed on the surfaces of the aluminum base materials **11**. The temperature of the low-temperature drying is preferably in a range of 25°C. to 30°C. and the pressure of the reduced-pressure drying is preferably in a range of 0.5 Pa to 1.0 Pa.

Through the Mixing Step **S01** and the Drying Step **S02**, the titanium powder particles **22** are dispersed and fixed to the outer surfaces of the aluminum base materials **11** as shown in FIG. 5 and the aluminum sintering material **20** according to the present embodiment is produced. The titanium powder particles **22** are preferably dispersed so that the intervals between the titanium powder particles **22** and **22** fixed to the outer surfaces of the aluminum base materials **11** are within a range of 5  $\mu\text{m}$  to 100  $\mu\text{m}$ .

Next, the porous aluminum sintered compact **10** is produced using the aluminum sintering material **20** obtained in the above-described manner.

In the present embodiment, for example, a long sheet-shaped porous aluminum sintered compact **10** having a width of 300 mm, a thickness in a range of 1 mm to 5 mm, and a length of 20 m is produced using a continuous sintering device **30** shown in FIG. 6.

The continuous sintering device **30** includes: a powder distributing apparatus **31** that uniformly distributes the aluminum sintering material **20**; a carbon sheet **32** that holds the aluminum sintering material **20** supplied from the powder distributing apparatus **31**; a transportation roller **33** that drives the carbon sheet **32**; a defatting furnace **34** that heats the aluminum sintering material **20** that is transported together with the carbon sheet **32** so as to remove the binder; and a sintering furnace **35** that heats and sinters the aluminum sintering material **20** from which the binder has been removed.

First, the aluminum sintering material **20** is distributed from the powder distributing apparatus **31** toward the carbon sheet **32** (Material Distributing Step **S03**).

The aluminum sintering material **20** distributed on the carbon sheet **32** spreads in the width direction of the carbon sheet **32** so as to have a uniform thickness and is shaped into a sheet shape while moving in the travelling direction **F**. At this time, since no load is applied, gaps are formed between the aluminum base materials **11** and **11** in the aluminum sintering material **20**.

Next, the aluminum sintering material **20** that is formed into a sheet shape on the carbon sheet **32** is loaded into the defatting furnace **34** together with the carbon sheet **32** and is heated at a predetermined temperature; and thereby, the binder is removed (Binder Removal Step **S04**).

In the Binder Removal Step **S04**, the aluminum sintering material is held in air atmosphere at a temperature in a range of 350°C. to 500°C. for 0.5 minutes to 30 minutes; and thereby, the binder in the aluminum sintering material **20** is removed. The heating temperature is preferably in a range of 350°C. to 450°C. and the holding time is preferably in a range of 10 minutes to 15 minutes. In the present embodiment, since the binder is used in order to fix the titanium powder particles **22** to the outer surfaces of the aluminum base materials **11** as described above, the amount of the binder is much smaller than that in a viscous composition and it is possible to sufficiently remove the binder within a short period of time.

Next, the aluminum sintering material **20** from which the binder has been removed is loaded into a sintering furnace **35** together with the carbon sheet **32** and is heated at a predetermined temperature so as to be sintered (Sintering Step **S05**).

In the Sintering Step **S05**, the aluminum sintering material is held in an inert gas atmosphere at a temperature in a range of 655°C. to 665°C. for 0.5 minutes to 60 minutes. The heating temperature is preferably in a range of 657°C. to 662°C. and the holding time is preferably set to be in a range of 1 minute to 20 minutes.

By using an inert gas atmosphere such as Ar gas and the like as the sintering atmosphere in the Sintering Step **S05**, it is possible to sufficiently decrease the dew point. A hydrogen atmosphere or a mixed atmosphere of hydrogen and nitrogen is not preferable since it is difficult to decrease the dew point. In addition, since nitrogen reacts with Ti so as to form TiN, the sintering acceleration effect of Ti is lost, which is not preferable.

Therefore, in the present embodiment, as the atmosphere gas, an Ar gas having a dew point of  $-50^{\circ}\text{C}$ . or lower is used. The dew point of the atmosphere gas is more preferably set to be in a range of  $-65^{\circ}\text{C}$ . or lower.

In the Sintering Step S05, since the aluminum sintering material is heated at a temperature in a range of  $655^{\circ}\text{C}$ . to  $665^{\circ}\text{C}$ ., which is approximate to the melting point of aluminum, the aluminum base materials 11 in the aluminum sintering material 20 are melted. Since oxide films are formed on the surfaces of the aluminum base materials 11, the molten aluminum is held by the oxide films and the shapes of the aluminum base materials 11 are maintained.

In addition, when the aluminum sintering material is heated at a temperature in a range of  $655^{\circ}\text{C}$ . to  $665^{\circ}\text{C}$ ., the oxide films are broken by the reaction with the titanium powder particles 22 which are fixed in the outer surfaces of the aluminum base materials 11 and the molten aluminum inside the aluminum sintering material is ejected outwards. The ejected molten aluminum reacts with titanium and thus a compound having a higher melting point is generated and solidified. Thereby, as shown in FIG. 7, a plurality of columnar protrusions 12 protruding outwards are formed on the outer surfaces of the aluminum base materials 11. At the tips of the columnar protrusions 12, the Ti—Al-based compound 16 is present, and the Ti—Al-based compound 16 suppresses (limits) the growth of the columnar protrusions 12.

In the case in which hydrogenated titanium is used as the titanium powder particles 22, the hydrogenated titanium is decomposed at a temperature within or in the vicinity of  $300^{\circ}\text{C}$ . to  $400^{\circ}\text{C}$ . and the generated titanium reacts with the oxide films on the surfaces of the aluminum base materials 11.

At this time, adjacent aluminum base materials 11 and 11 are bonded together by being integrated together in a molten state or solid-phase sintering through the columnar protrusions 12 on both of the aluminum base materials and, as shown in FIG. 1, the porous aluminum sintered compact 10 is produced in which a plurality of the aluminum base materials 11 and 11 are bonded together through the columnar protrusions 12. In addition, the Ti—Al-based compound 16 (the  $\text{Al}_3\text{Ti}$  intermetallic compound) is present in the bonding portions 15 at which the aluminum base materials 11 and 11 are bonded together through the columnar protrusions 12.

According to the aluminum sintering material 20, which is the present embodiment having the above-described features, when the aluminum sintering material is heated at a temperature of  $655^{\circ}\text{C}$ . to  $665^{\circ}\text{C}$ . which is near the melting point of aluminum in the Sintering Step S05, the oxide films formed on the surfaces of the aluminum base materials 11 are broken at the portions to which the titanium powder particles 22 are fixed and molten aluminum is ejected. When the ejected molten aluminum reacts with titanium and thus a compound having a higher melting point is generated and solidified, a plurality of columnar protrusions 12 protruding outwards are formed on the outer surfaces of the aluminum base materials 11. At this time, adjacent aluminum base materials 11 and 11 are bonded together by being integrated together in a molten state or solid-phase sintering through the columnar protrusions 12 on both of the aluminum base materials, and thus it becomes possible to produce the porous aluminum sintered compact 10 in which the a plurality of aluminum base materials 11 and 11 are bonded together through the columnar protrusions 12 as shown in FIG. 1.

As described above, since a structure is provided in which the aluminum base materials 11 and 11 are bonded together through the columnar protrusions 12 formed on the outer surfaces of the aluminum base materials 11, it is possible to obtain a porous aluminum sintered compact 10 having high porosity without separately carrying out a foaming step and the like. Therefore, it becomes possible to efficiently produce the porous aluminum sintered compact 10 according to the present embodiment at low cost.

Furthermore, unlike the case in which a viscous composition is used, a large amount of a binder is not present between the aluminum base materials 11 and 11, and thus it becomes possible to obtain a porous aluminum sintered compact 10 having a small shrinkage ratio during sintering and excellent dimensional accuracy.

In addition, since the oxide films are broken by titanium, the aluminum base materials 11 and 11 can be reliably bonded together and it is possible to obtain the porous aluminum sintered compact 10 having sufficient strength.

Furthermore, since the molten aluminum is solidified by titanium, it is possible to prevent the gaps between the aluminum base materials 11 and 11 from being filled with the molten aluminum, and it is possible to obtain the porous aluminum sintered compact 10 having high porosity.

In addition, in the aluminum sintering material 20 of the present embodiment, since the amount of the titanium powder particles 22 is set to be in a range of 0.5 mass % to 20 mass %, it is possible to form the columnar protrusions 12 at appropriate intervals on the outer surfaces of the aluminum base materials 11, and it is possible to obtain a porous aluminum sintered compact 10 having sufficient strength and high porosity.

In addition, in the present embodiment, since the aluminum fibers 11a and the aluminum powder 11b are used as the aluminum base materials 11, it becomes possible to control the porosity of the porous aluminum sintered compact 10 by adjusting the mixing ratio thereof.

In addition, in the porous aluminum sintered compact 10 of the present embodiment, since the porosity is set to be in a range of 30% to 90%, it becomes possible to provide a porous aluminum sintered compact 10 having the optimal porosity for a particular use.

In addition, in the present embodiment, since the intervals between the titanium powder particles 22 and 22 fixed to the outer surface of the aluminum base material 11 are set to be in a range of  $5\text{ }\mu\text{m}$  to  $100\text{ }\mu\text{m}$ , the intervals between the columnar protrusions 12 are optimized, and it is possible to obtain a porous aluminum sintered compact 10 having sufficient strength and high porosity.

Furthermore, in the present embodiment, since the fiber diameters of the aluminum fibers 11a, which are the aluminum base materials 11, are set to be in a range of  $40\text{ }\mu\text{m}$  to  $300\text{ }\mu\text{m}$ , the particle diameters of the aluminum powder 11b are set to be in a range of  $20\text{ }\mu\text{m}$  to  $300\text{ }\mu\text{m}$ , and the particle diameters of the titanium powder particles 22 are set to be in a range of  $1\text{ }\mu\text{m}$  to  $50\text{ }\mu\text{m}$ , it is possible to reliably disperse and fix the titanium powder particles 22 to the outer surfaces of the aluminum base materials 11 (the aluminum fibers 11a and the aluminum powder 11b).

Furthermore, according to the method for producing the aluminum sintering material 20 which is the present invention, since the Mixing Step S01 of mixing the aluminum base materials 11 and the titanium powder with a binder through spraying and the Drying Step S02 of drying a mixture obtained in the Mixing Step S01 are included, the titanium powder particles 22 are dispersed and fixed to the

## 11

outer surfaces of the aluminum base materials **11** and the above-described aluminum sintering material **20** can be produced.

Here, since low-temperature drying which is conducted at a temperature of 40° C. or lower or reduced-pressure drying which is conducted at a pressure of 1.33 Pa or less is applied in the Drying Step **S02**, it is possible to suppress (limit) the forming of thick oxide films on the surfaces of the aluminum base materials **11** in the Drying Step **S02**, and the sinterability of the aluminum sintering material **20** can be improved.

In addition, according to the method for producing a porous aluminum sintered compact which is the present embodiment, since the above-described aluminum sintering material **20** is used, a plurality of columnar protrusions **12** protruding outwards are formed on the outer surfaces of the aluminum base materials **11** and a plurality of the aluminum base materials **11** and **11** are bonded together through the columnar protrusions **12**. Therefore, it is possible to produce a porous aluminum sintered compact **10** having high porosity and sufficient strength.

In addition, in the present embodiment, since the continuous sintering device **30** shown in FIG. 6 is used, it is possible to continuously produce the sheet-shaped porous aluminum sintered compacts **10** and the production efficiency is greatly improved.

Furthermore, since the carbon sheet **32** is used as the holding body that holds the aluminum sintering material **20**, it is possible to favorably remove the porous aluminum sintered compact **10** from the carbon sheet **32** after sintering.

In addition, in the porous aluminum sintered compact **10** produced using the aluminum sintering material **20** according to the present embodiment, since the Ti—Al-based compound **16** is present in the bonding portions **15** between the aluminum base materials **11** and **11**, the oxide films formed on the surfaces of the aluminum base materials **11** are broken by the Ti—Al-based compound **16** and the aluminum base materials **11** and **11** are favorably bonded together. Therefore, it is possible to obtain a porous aluminum sintered compact **10** having sufficient strength.

Particularly, in the present embodiment, since Al<sub>3</sub>Ti is present as the Ti—Al-based compound **16** in the bonding portions **15** between the aluminum base materials **11** and **11**, the oxide films formed on the surfaces of the aluminum base materials **11** are reliably broken, the aluminum base materials **11** and **11** are favorably bonded together, and it is possible to ensure the strength of the porous aluminum sintered compact **10**.

In addition, in the present embodiment, since the aluminum base materials **11** are made of pure aluminum having a purity of 99.5 mass % or more and, furthermore, the aluminum base materials **11** are made of 4N aluminum having a purity of 99.99 mass % or more, it is possible to improve the corrosion resistance of the porous aluminum sintered compact **10**.

Furthermore, in the present embodiment, since the aluminum fibers **11a** and the aluminum powder **11b** are used as the aluminum base materials **11** and the mixing ratio of the aluminum powder lib is set to be in a range of 10 mass % or less, it is possible to obtain a porous aluminum sintered compact **10** having high porosity.

Thus far, the embodiment of the present invention has been described, but the present invention is not limited thereto and can be appropriately modified within the scope of the technical features of the invention.

For example, the method in which the porous aluminum sintered compacts are continuously produced using the

## 12

continuous sintering device shown in FIG. 6 has been described, but the method is not limited thereto and the porous aluminum sintered compact may be produced using other production devices.

In addition, in the present embodiment, the sheet-shaped porous aluminum sintered compact has been described, but the shape is not limited thereto and the porous aluminum sintered compact may be, for example, a bulk-shaped porous aluminum sintered compact produced through production steps shown in FIG. 8.

As shown in FIG. 8, the aluminum sintering material **20** is distributed from a powder distributing apparatus **131** that distributes the aluminum sintering material **20** toward the inside of a carbon container **132**; and thereby, bulk filling is carried out (Material Distributing Step). The carbon container **132** filled with the aluminum sintering material **20** is loaded into a defatting furnace **134** and is heated in air atmosphere; and thereby, a binder is removed (Binder Removal Step). After that, the aluminum sintering material is loaded into a sintering furnace **135** and is heated and held in an Ar atmosphere at a temperature in a range of 655° C. to 665° C.; and thereby, a bulk-shaped porous aluminum sintered compact **110** is obtained. Since the carbon container **132** having favorable mold release properties is used and the porous aluminum sintered compact shrinks approximately 1% during sintering, it is possible to remove the bulk-shaped porous aluminum sintered compact **110** from the carbon container **132** in a relatively easy manner.

## INDUSTRIAL APPLICABILITY

A porous aluminum sintered compact can be efficiently produced at low cost using the aluminum sintering material of the present invention and the produced porous aluminum sintered compact has a small shrinkage ratio during sintering, excellent dimensional accuracy, and sufficient strength. Therefore, the porous aluminum material of the present invention can be preferably used in production steps of porous aluminum sintered compacts that are applied to electrodes and current collectors in a variety of batteries, heat exchanger components, silencing components, filters, impact-absorbing components, and the like.

## DESCRIPTION OF THE REFERENCE NUMERALS

- 10, 110** POROUS ALUMINUM SINTERED COMPACT
- 11** ALUMINUM BASE MATERIAL
- 11a** ALUMINUM FIBER
- 11b** ALUMINUM POWDER
- 12** COLUMNAR PROTRUSION
- 15** BONDING PORTION
- 16** Ti—Al-BASED COMPOUND
- 20** ALUMINUM SINTERING MATERIAL
- 22** TITANIUM POWDER PARTICLE
- 32** CARBON SHEET (HOLDING BODY)
- 132** CARBON CONTAINER (HOLDING BODY)

The invention claimed is:

1. An aluminum sintering material that is used for producing a porous aluminum sintered compact in which a plurality of aluminum base materials are sintered together, the aluminum sintering material comprising:
  - the aluminum base materials; and
  - a plurality of titanium powder particles fixed to outer surfaces of the aluminum base materials, wherein

**13**

the titanium powder particles are composed of either one or both of metallic titanium powder particles and hydrogenated titanium powder particles,

the aluminum base materials are composed of:

aluminum fibers; or

5

aluminum fibers and aluminum powders, and

the aluminum base materials are made of pure aluminum having a purity of 99.5 mass % or more.

2. The aluminum sintering material according to claim 1, wherein an amount of the titanium powder particles is set 10 to be in a range of 0.5 mass % to 20 mass %.

3. The aluminum sintering material according to claim 1, wherein the aluminum base materials are composed of aluminum fibers and aluminum powders.

4. The aluminum sintering material according to claim 3, 15 wherein a ratio of the aluminum powder to the aluminum base materials is in a range of 1.0 mass % to 10.0 mass %.

5. The aluminum sintering material according to claim 1, wherein fiber diameters of the aluminum fibers are in a range 20 of 40  $\mu\text{m}$  to 300  $\mu\text{m}$ .

6. The aluminum sintering material according to claim 3, wherein particle diameters of the aluminum powder are in the range of 20  $\mu\text{m}$  to 300  $\mu\text{m}$ .

7. The aluminum sintering material according to claim 1, wherein particle diameters of the titanium powder particles 25 are in the range of 1  $\mu\text{m}$  to 50  $\mu\text{m}$ .

8. The aluminum sintering material according to claim 1, wherein an amount of the titanium powder particles is set to be in a range of 0.5 mass % to 20 mass %, and in a case in which the aluminum base materials are composed of the 30 aluminum fibers and the aluminum powders, the ratio of the aluminum powder is 5.0 mass % or less.

**14**